

## UNITED STATES PATENT OFFICE

OSCAR JAECK, DECEASED, LATE OF REINACH, NEAR BASEL, BY WOLFGANG JAECK, ADMINISTRATOR, OF BASEL, SWITZERLAND, AND FRITZ SCHÜTZ, OF BASEL, SWITZERLAND, ASSIGNORS TO THE FIRM OF SOCIETY OF CHEMICAL INDUSTRY IN BASLE, OF BASEL, SWITZERLAND

## PROCESS OF MAKING ACIDYL CELLULOSE

No Drawing. Application filed June 27, 1929, Serial No. 374,268, and in Switzerland July 13, 1928.

Hitherto vegetable fibers have been immunized to direct dyeing dyestuffs by means of acetic anhydride by treating the fibers for a long time with the acylating agent, to which a catalyst has been added.

The present invention essentially simplifies this process, in that the textile to be immunized is first treated with a heavy metal salt of a strong acid, such as copper sulfate or copper sulfate in the presence of a very small amount of sulfuric acid, as is the case with crude copper sulfate, and then acylated by means of an acylating mixture. The advantage of the invention resides in the substantial shortening of the acylating operation, which is reduced by the invention from several hours or days to a fraction of an hour.

The following example illustrates the invention:—

20 1 kilo of the usual prepared cotton is impregnated with a solution of crude copper sulfate of 1 per cent. strength and then hydro-extracted and dried. The goods are then immersed in 10 parts of acetic anhydride at the 25 temperature of the water-bath. At the end of half-an-hour, the immunizing is complete, whereupon the goods are removed, hydro-extracted, rinsed and dried.

What we claim is:—

30 1. A process for immunizing vegetable fibers to direct dyeing dyestuffs by means of acetic anhydride, wherein the vegetable fiber is first treated with a solution of copper sulfate in the presence of a very small amount 35 of sulfuric acid and then, after preliminary drying, acylated by means of an acylating agent.

2. A process for immunizing vegetable fibers to direct dyeing dyestuffs by means of 40 acetic anhydride, wherein the vegetable fiber is first treated with a solution of copper sulfate in the presence of a very small amount of sulfuric acid and then, after preliminary drying, acylated by means of acetic anhydride.

In witness whereof we have hereunto signed our names this 15th day of June, 1929.

WOLFGANG JAECK,  
Administrator of the Estate of Oscar Jaeck,  
Deceased.

FRITZ SCHÜTZ.

50

55

60

65

70

75

80

85

90